# EUROPEAN PATENT SPECIFICATION

(11) **EP 0 327 413 B1**
(45) Date of publication and mention of the grant of the patent: **03.11.1993**
(21) Application number: 89400054.6
(22) Date of filing: 09.01.1989
(51) Int. Cl.: D06Q 1/00, C11D 3/395, D06B 11/00

(54) **Method for producing pattern on denim product**
Verfahren zum Herstellen von Mustern auf jeansartigen Produkten
Méthode pour produire des dessins sur des produits en jean

(30) Priority: 08.01.1988 JP 2702/88; 13.02.1988 JP 17921/88; 13.07.1988 JP 175578/88; 08.11.1988 JP 282685/88
(43) Date of publication of application: 09.08.1989
(73) Proprietor: Yamate, Masato, Fukuyama-shi Hiroshima-ken (JP)
(72) Inventor: Yamate, Masato, Fukuyama-shi Hiroshima-ken (JP)
(74) Representative: Netter, André

(56) References cited:
- EP-A- 0 303 120
- BE-A- 438 763
- BE-A- 905 631

## Description

The present invention relates to methods for producing a pattern on a denim product including woven fabric and raw cloth, such as a pair of trousers and jackets, etc.

Denim products (or blue jeans) are in fashion these days as trousers or jackets. They are made of relatively thick fabrics, either twilled or flatly woven with dark blue threads as weft, and white threads as warp.

In order to produce a pattern on these products by means of the so-called "Chemical Wash Method", the fabrics are put into a drum along with a plurality of pumices impregnated with a bleaching solution, such as, calcium hypochlorite solution. And, as the drum is rotated, the denim products are scrubbed with the pumices, thereby creating the so-called "pepper-and-salt", mottled pattern on the scrubbed portions. On the other hand, in accordance with the so-called "Chemical Bleach Method", such fabrics are immersed and agitated in a bleaching solution, such as, calcium hypochlorite solution for a prescribed period of time, thereby decolorizing (or bleaching) the fabric as a whole.

As mentioned above, the conventional pattern given to the denim products obtainable by the Chemical Wash Method is constituted by a multitudes of mottles which are irregularly situated all over the fabric. Moreover, the latter Chemical Bleach Method is simply capable of decolorizing the whole fabric unifomly. Thus, the conventional pattern producing method is incapable of freely generating unique and individual patterns (or designs) on denim products.

The present invention is in the first place a method for producing a pattern on a denim product comprising the steps of :
providing a paste-like material including albumen or yolk or mixture thereof ;
drawing a desired pattern on the denim product with a bleach inhibiting agent comprising said paste-like material ;
putting said product into a drum with a plurality of pumices impregnated with a bleaching solution ; and
rotating said drum for a prescribed period of time ;
whereby said pattern remains in dark blue in contrast with the other portion as result of the scrubbing between the denim product and the pumices.

The present invention is secondly a method for producing a pattern on a denim product comprising the steps of :
providing a paste-like material including albumen or yolk or mixture thereof ;
drawing a desired pattern on the denim product with a bleach inhibiting agent comprising said paste-like material ;
drying said denim product ; and
putting it in a bleaching solution and agitating it for a prescribed period of time ;
whereby the portion where the pattern has been drawn remains in dark blue in contrast with the other portion.

What can be used as the bleach inhibiting agent includes a paste-like material including albumen or yolk or mixture thereof; or paste itself (or starch); or wax, which can provide resistance to the bleaching function of the bleaching solution.

The bleaching solution may be selected from the group of calcium hypochlorite, sodium hypochlorite and potassium permanganate, etc. The appropriate concentration of such a bleaching solution is well known in the industry.

In the above-mentioned second method, in order to prolong the retention of the bleach inhibiting agent with the fabric immersed in the bleaching solution, it is useful, after drying the denim product, to apply a coating on the pattern comprising principally albumen. For the same purpose, the bleach inhibiting agent may include paint (water-soluble or oil-soluble).

On the other hand, if the bleaching solution includes acetic acid, the rate of bleaching of the bleaching solution may be increased substantially; and the necessary bleaching may be accomplished in a shorter period of time. Then, applying additional coating or inclusion of paint in the agent as mentioned above, may be done away with.

The present invention is thirdly a method for producing a pattern on a denim product comprising the steps of:
drawing a desired pattern on the denim product with a first solution which is a mixture of varnish and alcohol for promoting bleach of denim products when applied thereon ;
putting said denim product in a second bleaching solution and agitating it for a prescribed period of time;
whereby the portion where the pattern has been drawn may be decolorized faster than the other portion.

The first solution functions to promote the bleaching of the portion where the solution has been applied to make said portion whiter than the rest.

If the third method includes the step of drawing a pattern on the denim product with a solution or paste-like material including a bleaching agent before or after drawing the pattern with the first solution, the portion where the pattern has been drawn additionally may be made even whiter than the portion where the pattern was drawn with the first solution.

It is to be understood that the methods of this invention may be used in combination on the same product.

The present invention uses a bleach inhibiting agent for denim products when applied thereon including albumen or yolk or mixture thereof ; and a bleach promoting agent for denim products when applied thereon comprising a mixture solution of varnish and alcohol. The paste-like material may preferably be mixed in alcohol (ethyl or methyl), since alcohol functions to enhance penetration of the agent into the denim fabric ; and it also functions as an antiseptic. If necessary, additional antiseptics may be added.

A desired pattern may be drawn by means of a brush or a so-called "screen painting" depending upon the hardness (or viscosity) of the bleach inhibiting or promoting agents. In order to change the hardness and/or reduce the cost of the agents, fillers in the form of powder, such as, wheat flour, pulverized egg shells or ashes may preferably be added.

Needless to say, the denim products thus given patterns are to be washed; dried; and pressed to render them in their final forms.

Figs. 1 to 3 are block diagrams showing three different methods of pattern producing according to the present invention, respectively.

Figs. 4 and 5 show denim products which have been given patterns according to the first and second methods of the present invention.

Figs. 6 and 7 illustrate how a desired pattern may be produced according to the third method of the present invention.

### Example 1

As shown in Fig. 4, the pattern m was drawn on a pair of trousers 1 with a brush (not shown) utilizing foamed albumen (or egg white) as a bleach inhibiting agent. 25 pairs of the trousers thus given the pattern were put into a drum. A prescribed amount of pumices (about 40 kg) impregnated with a calcium hypochlorite solution (effective chlorine 12 %) were then put into the drum. The drum was rotated for about 15 minutes at 30 r.p.m clockwise and counter-clockwise.

As result of the scrubbing of the fabric with the pumices, those portions excepting the portions where the pattern was drawn became pepper-and-salt; however, the portions where the pattern was drawn as above-mentioned remained in dark blue in striking contrast as shown in Fig. 4.

### Example 2

As shown in Fig. 5, the pattern n was drawn on a jacket 2 with a brush (not shown) utilizing, as a bleach inhibiting agent, a solution of paste made from wheat flour. 20 jackets thus given the pattern were put into a drum. A prescribed amount of pumices (about 35 kg) impregnated with a calcium hypochlorite solution were then put into the drum. The drum was rotated for about 20 minutes (44 r.p.m) clockwise and counter-clockwise.

As result of the scrubbing of the fabric with the pumices, those portion excepting the portions where the pattern was drawn became pepper-and-salt; however, the portions where the pattern was drawn remained in dark blue in striking contrast as shown in Fig. 5. Similar results were obtained using yolk (or egg yellow), or a mixture of albumen and yolk, or wax as the bleach inhibiting agent.

### Example 3

As shown in Fig. 4, the pattern m was drawn on a pair of trousers 1 by means of a so-called "screen painting" utilizing, as the bleach inhibiting agent, a paste prepared by mixing and agitating albumen and pulverized egg shells with wheat flour and about 10% (by weight) water-soluble paint (color: blue) in an industrial alcohol.

The produce was dried in a drier for a prescribed period of time. Taking the product out from the drier, a coating agent comprising 100% albumen was applied to the pattern and the product was dried again.

After drying, the product was put into a 6 % (by volume) solution of calcium hypochlorite and agitated for about 7 minutes.

As a result, the fabric as a whole was decolorized in white; but those portions where the pattern was drawn remained in dark blue in striking contrast with the other portions as shown in Fig. 4.

### Example 4

As shown in Fig. 5, the pattern n was drawn on a jacket 2 with a brush (not shown) utilizing a paste having an appropriate hardness prepared by mixing and agitating albumen and pulverized egg shells with wheat flour in an industrial alcohol added with about 10% water-soluble paint (color: green). The product was dried in a drier for a prescribed period of time.

Taking the product out from the drier, a coating agent comprising 95% albumen and 5% gelatine was applied to the pattern and the product was dried again.

After drying, the product was put into a 7 % solution of calcium hypochlorite and agitated for about 10 minutes.

As a result, the fabric as a whole was decolorized in white; but those portions where the pattern was drawn remained in dark blue in striking contrast with the other portions as shown in Fig. 5.

### Example 5

As shown in Fig. 6, the pattern p was drawn on a jacket 2' of denim with a brush 3 utilizing a first solution 4 which is a mixture of varnish and alcohol with a ratio of approximately 1 to 1.

Next, the jacket 2′ was put into a second solution comprising water (1 part), calcium hypochlorite (0.015 to 0.10 part) and acetic acid (0.002 to 0.07 part); and agitated for a prescribed period of time ( 2 to 6 minutes). The concentration of acetic acid itself was 60.05 %. Those portions where the first solution 4 was applied were decolorized faster than the rest, thereby producing the desired pattern.

Thereafter, the product 2′ was taken out; washed and dried to obtain a final product shown in Fig. 7.

It is to be noted that as the proportion of alcohol becomes larger relative to varnish, it becomes easier to draw a pattern; however, if it becomes too large, a clear pattern drawing will become difficult. On the other hand, if the proportion is reversed, the resultant pattern may be made clearer; however, it should be noted that the initial pattern drawing could become somewhat difficult. Thus, the proportion should be adjusted between about 30 to 70 %.

The addition of acetic acid in the second solution of calcium hypochlorite serves to accelerate the decolorization; as the amount of acetic acid is increased, the desired decolorization will be accomplished quicker. However, since too much acetic acid will cause the resultant denim products to discolor to an undesirable degree, the amount of acetic acid should be adjusted within about 10%. Furthermore, the addition of acetic acid may be done away with.

The denim products are to be agitated in the bleaching solution as above mentioned for about 2 to 8 minutes. The resultant shade of pattern may be clearer when subjected to agitation for a shorter time. If subjected to agitation for a longer time, the pattern will tend to become dimmer; and it is to be noted that the fabric itself could be damaged.

### Example 6

A paste-like material was prepared by mixing and agitating albumen and a paste made from wheat flour with a proportion of 1 vs 0.5.

### Example 7

A paste-like material was prepared by mixing and agitating 1.00 yolk, 0.60 albumen and 0.40 wheat flour paste.

### Example 8

A paste-like material was prepared by mixing and agitating 0.375 yolk, 0.25 albumen, 0.125 pulverized egg shells and 0.25 wheat flour paste.

The paste-like materials as shown in Examples 6 to 8 were found useful as the bleach inhibiting agents to be used in the present invention, although the agent in Example 7 produced somewhat dimmer design in comparison with the other Examples.

## Claims

1. A method for producing a pattern on a denim product comprising the steps of :
- providing a paste-like material including albumen or yolk or mixture thereof ;
- drawing a desired pattern (m, n) on the denim product (1, 2) with a bleach inhibiting agent comprising said paste-like material;
- putting said product into a drum with a plurality of pumices impregnated with a bleaching solution ; and
- rotating said drum for a prescribed period of time ;
whereby said pattern remains in dark blue in contrast with the other portion as result of the scrubbing between the denim product and the pumices.

2. A method for producing a pattern on a denim product comprising the steps of:
- providing a paste-like material including albumen or yolk or mixture thereof ;
- drawing a desired pattern (m, n) on the denim product (1, 2) with a bleach inhibiting agent comprising said paste-like material ;
- drying said denim product ; and
- putting it in a bleaching solution and agitating it for a prescribed period of time ;
whereby the portion where the pattern has been drawn remains in dark blue in contrast with the other portion.

3. The method of claim 1 or 2 wherein the bleaching solution includes acetic acid.

4. The method of claim 2 further including, after the drying step of the denim product, the steps of coating the portion where the pattern was given by a coating agent comprising principally albumen, and drying the denim product.

5. The method of claim 1 or 2 wherein the paste-like material includes paint.

6. The method of claim 1 or 2 wherein the paste-like material includes powdery filler.

7. A method for producing a pattern on a denim product comprising the steps of:
- drawing a desired pattern (p) on the denim product (2') with a first solution (4) which is a mixture of varnish and alcohol for promoting bleach of denim products when applied thereon ;
- putting said denim product in a second bleaching solution and agitating it for a prescribed period of time ;
whereby the portion where the pattern has been drawn may be decolorized faster than the other portion.

8. The method of claim 7 further including the step of drawing a pattern on the denim product with a solution or paste-like material including a bleaching agent before or after drawing the pattern with the first solution.

9. The method of claim 7 or 8 wherein the proportion of varnish and alcohol in the first solution is about 1 to 1.

10. The method of claim 7 or 8 wherein the second solution includes acetic acid.

## Patentansprüche

1. Verfahren zur Herstellung eines Musters auf einem Denim-Produkt, umfassend folgende Schritte :
- Bereitstellung eines pastenartigen Materials, das Eisweiss oder Eigelb oder eine Mischung beider Stoffe enthält,
- Zeichnen eines gewünschten Musters (m, n) auf das Denim-Produkt (1, 2) mit einem Bleichhemmittel, das das genannte pastenartige Material enthält,
- Einlegen des genannten Produkts in eine Trommel zusammen mit mehreren, mit einer Bleichlösung imprägnierten Bimssteinen und
- Drehen der genannten Trommel für eine vorbestimmte Zeit,
wobei das genannte Muster in Gegensatz zum übrigen Teil beim Scheuern zwischen Denim und Bims dunkelblau bleibt.

2. Verfahren zur Herstellung eines Musters auf einem Denim-Produkt, umfassend folgende Schritte :
- Bereitstellung eines pastenartigen Materials, das Eiweiss oder Eigelb oder eine Mischung beider Stoffe enthält,
- Zeichnen eines gewünschten Musters (m, n) auf das Denim-Produkt (1, 2) mit einem Bleichhemmittel, das das genannte pastenartige Material enthält,
- Trocknen des genannten Denim-Produkts und
- Einlegen des Produkts in eine Bleichlösung und Bewegen des Produkts in der Lösung für eine vorbestimmte Zeit,
wobei der Teil mit dem aufgezeichneten Muster im Gegensatz zum übrigen Teil dunkelblau bleibt.

3. Verfahren gemäss Anspruch 1 oder 2, dadurch gekennzeichnet, dass die Bleichlösung Essigsäure enthält.

4. Verfahren gemäss Anspruch 2, nach dem Trocknen des Denim-Produkts weiterhin folgende Schritte umfassend: Beschichtung des bemusterten Teils mit einem Beschichtungmittel, das hauptsächlich Eiweiss enthält, und Trocknen des Denim-Produkts.

5. Verfahren gemäss Anspruch 1 oder 2, dadurch gekennzeichnet, dass das pastenartige Material Farbstoff enthält.

6. Verfahren gemäss Anspruch 1 oder 2, dadurch gekennzeichnet dass das pastenartige Material ein pulverförmiges Füllmittel enthält.

7. Verfahren zur Herstellung eines Musters auf einem Denim-Produkt, umfassend folgende Schritte:
- Zeichnen eines gewünschten Musters (p) auf das Denim-Produkt (2) mit einer ersten Lösung (4), die eine Mischung aus Lack und Alkohol darstellt und bei Aufbringen auf Denim-Produkts das Bleichen derselben fördert,
- Einlegen des genannten Denim-Produkts in eine zweite Bleichlösung und Bewegen des Produkts in der Lösung fur eine vorbestimmte Zeit,
wobei der Teil mit dem aufgezeichneten Muster schneller entfärbt werden kann als der übrige Teil.

8. Verfahren gemäss Anspruch 7, desweiteren umfassend den folgenden Schritt : vor oder nach dem Aufzeichnen des Musters mit der ersten Lösung Aufzeichnen eines Musters auf das Denim-Produkt mit einer Lösung oder einem pastenartigen Material, das ein Bleichmittel enthält.

9. Verfahren gemäss Anspruch 7 oder 8, dadurch gekennzeichnet, dass das Verhältnis von Lack zu Alkohol in der ersten Lösung bei ca. 1:1 liegt.

10. Verfahren gemäss Anspruch 7 oder 8, dadurch gekennzeichnet, dass die zweite Lösung Essigsäure enthält.

## Revendications

1. Procédé pour produire un dessin sur un produit en jean, comprenant les étapes consistant à :
- prévoir une matière pâteuse contenant de l'albumine ou du jaune d'oeuf ou un mélange de ceux-ci;
- tracer un dessin désiré (m,n) sur le produit en jean (1,2) avec un agent inhibiteur de blanchiment comprenant ladite matière pâteuse;
- mettre ledit produit dans un tambour avec une multiplicité de pierres ponce imprégnées d'une solution de blanchiment; et
- faire tourner ledit tambour pendant une période de temps prescrite;
grâce à quoi ledit dessin reste bleu foncé contrairement à la partie restante par suite de la friction entre le produit en jean et les pierres ponce.

2. Procédé pour produire un dessin sur un produit en jean, comprenant les étapes consistant à :
- prévoir une matière pâteuse contenant de l'albumine ou du jaune d'oeuf ou un mélange de ceux-ci;
- tracer un dessin désiré (m,n) sur le produit en jean (1,2) avec un agent inhibiteur de blanchiment comprenant ladite matière pâteuse;
- sécher ledit produit en jean; et
- le mettre dans une solution de blanchiment et l'agiter pendant une période de temps prescrite;
grâce à quoi la partie où le dessin a été tracé reste bleu foncé, contrairement à la partie restante.

3. Procédé selon l'une des revendications 1 et 2, dans lequel la solution de blanchiment contient de l'acide acétique.

4. Procédé selon la revendication 2, comprenant en outre, après l'étape de séchage du produit en jean, les étapes consistant à revêtir la partie où le dessin a été formé par un agent de revêtement comprenant principalement de l'albumine, et sécher le produit en jean.

5. Procédé selon l'une des revendications 1 et 2, dans lequel la matière pâteuse contient de la peinture.

6. Procédé selon l'une des revendications 1 et 2, dans lequel la matière pâteuse contient une charge pulvérulente.

7. Procédé pour produire un dessin sur un produit en jean, comprenant les étapes consistant à :
- tracer un dessin désiré (p) sur le produit en jean (2') avec une première solution (4) qui est un mélange de vernis et d'alcool pour activer le blanchiment de produits en jean lorsqu'elle y est appliquée;
- mettre ledit produit en jean dans une seconde solution de blanchiment et l'agiter pendant une période de temps prescrite;
grâce à quoi la partie où le dessin a été tracé peut être décolorée plus vite que la partie restante.

8. Procédé selon la revendication 7, comprenant en outre l'étape consistant à tracer un dessin sur le produit en jean avec une solution ou une matière pâteuse contenant un agent de blanchiment avant ou après le tracé du dessin avec la première solution.

9. Procédé selon l'une des revendications 7 et 8, dans lequel la proportion de vernis et d'alcool dans la première solution est environ 1 pour 1.

10. Procédé selon l'une des revendications 7 et 8, dans lequel la seconde solution contient de l'acide acétique.
